

## UNITED STATES PATENT OFFICE.

ARMIN PEETZ, OF ALFELD, GERMANY.

## MANUFACTURE OF CHEMICAL WOOD PULP.

No Drawing. Application filed January 29, 1925; Serial No. 5,629, and in Germany April 30, 1924.

This invention relates to improvements in the manufacture of chemical wood pulp, and in particular to the manufacture of so-called sulphite fiber by the cooking of 5 wood chips and of similar vegetable fibers by bisulphite-solutions, usually of lime, magnesia and the like, and it is intended to devise means for facilitating the cooking process, and for improving the quality, 10 colour and strength of the fiber thereby obtained. As is well known, the usual procedure of manufacturing chemical pulp from wood or similar vegetable fibrous material is characterized by the fact that the 15 raw material in the comminuted condition is boiled for a sufficient length of time by bisulphite solutions. In this cooking process a certain maximum pressure according to the different requirements of the 20 particular case should not be exceeded. Whenever this admissible limit of pressure is exceeded in the cooking operation which is always effected by passing steam into the digesters, a reduction of pressure is produced by opening a valve provided in the 25 upper portion of the digester. Through this valve a certain proportion of the gaseous sulphurous acid and corresponding, though small quantities of the liquid contents of the digester are ejected, and the 30 pressure in the interior of the digester is lowered below the admissible maximum pressure, which maximum, however, is again exceeded after some time, and is again followed by an opening of the valve and ejec- 35 tion of sulphurous acid with a correspond- 40 ing reduction of pressure. This procedure is continued, until the pressure in the digester has ceased to go beyond the admissible highest limit. In this stage the digester is allowed to remain quiet for some time, and then the contents of the digester are boiled to the finish with the continued 45 admission of steam. The increase of pressure in the digester is effected by the sulphurous acid, liberated by the increase of 50 temperature and by the mechanical agitation of the liquor, and by the pressure of the saturated steam corresponding to the particular 55 temperature, and by the quantity of air liberated from the pores of the wood during the cooking process. The heating of the entire contents of the digester to the end-temperature of, for instance, say 138 60 degrees C. necessitates the consumption of a considerable amount of steam, and it is

well known that the commercial success of the manufacture of wood pulp depends chiefly upon the quantities of steam required.

In accordance with my invention it has been ascertained that it is possible to reduce the amount of steam required to a fraction of the amount necessary according to the previous method, and yet to produce a pulp of a better quality than in the ordinary process by letting corresponding amounts of the liquor flow away through a valve at the bottom of the digester for the reduction of pressure required, instead of 60 causing the liberated sulphurous acid to escape through a valve provided at the top of the digester. The amount of liquor which is removed in this manner, contains approximately the same quantity of sulphurous acid, which is allowed to escape in the previous method by the relieving operation through the upper valve. The removal of liquor is repeated as many times as may be required for the reduction of the interior 65 pressure. By this gradual withdrawal of a considerable portion of the liquor originally charged upon the wood, a considerable saving of steam is effected in view of the fact that the amount of liquor which has been 70 gradually withdrawn from the digester, and consequently does not need to be heated to the higher temperature.

With a view of producing an unobjectionable especially high-grade pulp of particu- 75 larly white colour it is of importance to expel the air as completely as possible from the digester before the cooking is finished. This requirement is accomplished in accordance with my invention by the opening 80 of the upper venting cock at a certain stage of the process. If, after this venting operation the interior pressure in the digester does not exceed the sum of the pressure of the sulphurous acid and steam at the re- 85 spective temperature, this will be a reliable indication that no air is left in the digester. Unless this result is accomplished with one venting operation, the venting should be repeated. There is no remarkable loss of sul- 90 phurous acid connected therewith, inasmuch as by the preceding withdrawal of consider- 95 able portions of the liquor from the digester the liberation of free sulphurous acid has been reduced to a minimum.

After the venting operation the cooking process is carried through in the usual man-

ner, and upon any excessing of the admissible maximum pressure the required reduction of pressure is always produced by the removal of a corresponding amount of liquor through the discharge valve at the bottom.

*Example 1.*

Liquor is charged in the usual manner into 10 the digester which has been supplied with wood, and after compressing and steaming the wood in order to expel the air then more liquor is subsequently pumped in until a certain pressure is reached when the acid- 15 pump is stopped. After that steam is admitted, and the pressure in the digester will increase to 4.2 atmospheres. By opening the bottom valve liquor is discharged until the excess pressure drops to 1.2 atmospheres. 20 This drop of pressure from 4.2 to 1.2 atmospheres is continued until a temperature of about 105 degrees C. is reached. Then the steam is shut in for say about 1½ hours, with a simultaneous short venting by the 25 top-valve, until the cooking pressure is equal to the sum of the pressure of sulphurous acid and the pressure of saturated steam corresponding to 105 degrees C., which partial pressures have been found by tests. 30 Then the steam is again admitted, and the reduction of pressure from 4.2 to 3.2 atmospheres is produced by withdrawal of liquor, until the final temperature of 138 degrees is reached. All further steps are carried out 35 in the usual manner.

It should be pointed out that the process according to this invention is not restricted to the manufacture of pulp by the sulphite process, but it may also be employed, when 40 the digestion is effected by alkalis or neutral salts. Nor is the invention restricted to the

precise scheme of procedure and the elements described, but modifications may occur in accordance with local requirements and the convenience of the operator, and 45 without deviating from the spirit of my invention, as pointed out in the claims, hereunto appended.

I claim:

1. The process of manufacturing chemical 50 wood pulp and the like from wood and similar material by digestion, which consists in keeping the digestion pressure at the admissible limit and reducing any excess of pressure by withdrawing portions of the liquor, 55 until the desired temperature is reached, then removing the liberated air from the top of the digester, finishing the digestion, and preventing any further substantial rise of pressure.

2. The process of manufacturing chemical 60 wood pulp by digestion, which consists in reducing any excess of pressure by withdrawing portions of the liquor until the desired temperature is reached, then removing 65 the liberated air from above the liquid, and reducing any excess of pressure by withdrawal of further quantities of liquor.

3. The process of manufacturing chemical 70 wood pulp by digestion with a liquor, which consists in reducing excess of pressure beyond the admissible limit by withdrawing portions of the liquor until a temperature of about 105 degrees centigrade is obtained, then removing the liberated air from above the 75 liquid, then finishing the digestion, and regulating the pressure by withdrawal of liquor during the finishing operation.

In testimony whereof I have signed this specification.

DR. ARMIN PEETZ.